

June 22, 1926.

1,589,730

E. H. WILLIAMS

METHOD AND APPARATUS FOR CASTING STEEL INGOTS

Filed Jan. 24, 1921

2 Sheets-Sheet 1



Fig. 1.



Fig. 2.



Fig. 3.

Inventor

Edward H. Williams

By his Attorney

George Ramey

June 22, 1926.

E. H. WILLIAMS

1,589,730

METHOD AND APPARATUS FOR CASTING STEEL INGOTS

Filed Jan. 24, 1921

2 Sheets-Sheet 2



Fig. 4.



Fig. 5.



Fig. 6.



Fig. 7.

Inventor

Edward H. Williams

By his Attorney

George Ramsey

## UNITED STATES PATENT OFFICE.

EDWARD H. WILLIAMS, OF SHARON, PENNSYLVANIA, ASSIGNOR TO VALLEY MOULD & IRON CORPORATION, OF SHARPSVILLE, PENNSYLVANIA, A CORPORATION OF NEW YORK.

## METHOD AND APPARATUS FOR CASTING STEEL INGOTS.

Application filed January 24, 1921. Serial No. 439,357.

This invention relates broadly to metallurgy and more specially to a method and apparatus for casting horizontal ingots from "dead melted" steel.

5 The principal object of the present invention is the method and apparatus of casting horizontal ingots from "dead melted" steel by providing a hot member in contact with one end of the ingot during 10 pouring and cooling.

A still further object of the present invention is the method and apparatus of casting steel ingots from "dead melted" steel wherein a heated runner is provided 15 adjacent one end of the ingot in such manner as to prevent chilling of one end of the ingot during pouring, thereby permitting molten steel to be supplied until the steel is set, thus preventing formation of pipes or 20 cavities in the ingot.

A still further object of the present invention is a method and apparatus of casting steel ingots in horizontal molds by providing a runner adjacent one end of the 25 mold and which runner is provided with a plurality of openings arranged in such manner that substantially the same volume of steel issues from the upper and lower openings into the mold during the pouring 30 operation.

A still further and important object of the present invention is the method and apparatus of casting horizontal steel ingots which comprises arranging runner openings adjacent one end of the matrix end of the 35 mold in such manner that a plurality of inlets lead from the runner to the matrix and with the upper inlets being of larger cross-sectional area than the lower inlets.

40 A still further and important object of the present invention is an ingot mold for casting horizontal steel ingots, which mold is provided with an opening adjacent one end thereof adapted to receive a runner tile of such size as to comprise the majority of the end wall of the matrix portion of the mold when the runner tile is in position.

A still further and primary object of the present invention is an article of manufacture comprising a runner tile for use in

casting horizontal ingots, which runner tile is of relatively wide width to prevent chilling of the steel adjacent the runner tile during the pouring operation and wherein said runner tile is adapted to be standardized so that said tile may be interchangeable with any one of a plurality of molds.

55 Another object of the present invention is an article of manufacture comprising a runner tile for use in casting horizontal steel ingots and wherein the runner tile and fountain are integral and formed in such manner that the fountain extends substantially to the uppermost inlet opening adapted to lead into the mold matrix.

60 A still further object of the present invention is the provision of a runner tile for use in casting horizontal steel ingots, which tile comprises an earthen product preferably of porous texture and adapted to have 65 large heat absorbing capacity whereby the runner tile may be heated very hot before being set so as to give off heat during the pouring operation and prevent chilling of the steel being poured.

70 Other and further objects of the present invention will in part be obvious and will in part be pointed out hereinafter by reference to the accompanying drawings forming a part of this application and wherein 75 like parts are indicated by like characters throughout the several figures thereof.

75 Realizing that the present invention may be embodied in constructions other than those specifically shown and described it is desired that the disclosure herewith shall be considered as illustrative and not in the limiting sense.

80 Figure 1 of the drawings illustrates a horizontal section through a two-part mold having a vertical separation plane with the view taken on the separation plane and showing the runner tile in section.

85 Figure 2 is a view illustrating the pouring action.

90 Figure 3 is a view illustrating shrinkage after the ingot is cold and showing the shrinkage exaggerated to more clearly illustrate the same.

95 Figure 4 is a cross section of the mold at 100

one end of the mold and through the runner tile recess on line 4—4 Figure 1 with the runner tile of the mold.

Figure 5 is a cross-section on line 5—5  
5 Figure 1.

Figure 6 is a cross-section of the runner tile.

Figure 7 is a perspective view of the runner tile shown in Figure 6.

10 The present invention relates more specially to the production of ingots from "dead melted" or "piping" steel, such as steel from which the free gases have been largely eliminated and which pours without bubbling  
15 or boiling as is the usual action of ordinary or "wild" steel. Alloy or high carbon steels which are usually used for special purposes, for example, high speed tool steel, rail, or the like, are usually "dead melted" steels.  
20 Such steels may comprise alloys of titanium, vanadium, chromium, tungsten, nickel, combined carbon etc. This type of steel usually pours "dead" and when made into ingots has a considerable tendency to  
25 pipe. Because of the special purposes for which such steel is used any portion of the ingot which has pipes must be scrapped. It is customary in the production of commercial shapes from steel of this type, for example, high speed tool steel to subject the ingots to elaborate processes of manufacture to determine and eliminate these troublesome pipes. Heretofore it has been customary to cast small vertical ingots from  
30 this type of steel. These ingots are usually cropped in rough to such a point as the operator believes will eliminate the majority of the pipes. Ingots of this steel are usually subjected to processes of annealing, hammering, pickling, grinding, chipping etc., to get rid of pipes. For example, an ingot of high speed tool steel will be first annealed; then cogged, hammered, or rolled into an elongated form of general rectangular shape; then the seams are ground out. The bloom thus formed is pickled with acid, then cropped. If any pipes show the bloom is again cropped. This operation is continued until all evidences of pipes disappear. The bloom or billet is then annealed again and is then rolled or shaped into the final form, usually a bar, which is again inspected, annealed and defects cut out, and the remaining portion is ready for the market. Often times defects in the original ingot show up in the final shape so that a large portion of the final form even may be cropped and discarded as scrap. This type of steel pipes so badly that in the average run of ingots only a relatively small percentage is manufactured into final product, and a relatively large percentage is thrown aside as scrap. This very greatly increases the cost of producing such steel.

65 The present invention overcomes the dif-

ficulties of the known art and produces what is known in the art as a "perfect ingot" of which substantially all portions thereof may be manufactured into finished product. Preferably this invention is carried out in 70 inclined horizontal chill molds with runner tiles at one end thereof. These tiles preferably are arranged to produce vertical agitation in the steel in the mold during pouring and this may be accomplished by a plurality of openings in the runner tile. Where cold runner tiles are used in casting this type of steel the ingot may appear substantially solid but there is a liability of a small pipe leading from the upper opening into the ingot downwardly at an angle about double the angle of inclination of the axis of the mold. This liability is completely overcome by heating the runner tile and supplying sufficient fresh steel to follow up and fill 75 all tendencies to cavitate. It is also desirable that the runner tile have the fountain integral with the body of the tile with the funnel opening of the fountain leading substantially to the upper inlet opening in the body of the tile and with the lower inlet opening in the runner tile of less diameter than the upper opening. When the tile is so constructed substantially the same amount of steel enters the mold matrix from each 80 opening during pouring. This insures the steel entering through the lower opening spouting into the mold with considerable force and velocity while the steel entering through the upper opening will fall downwardly upon the lower stream, thereby producing a churning action which will continue while the mold is rapidly being filled. Since the mold is a chill mold the steel farthest from the inlet cools first and the cooling 85 action progresses from the remote end toward the inlet opening so that the portion of the ingot against the wide hot runner is last to freeze. Consequently the freezing or shrinking steel is continually fed on the inside or core portion by liquid or molten steel, up to the final instant of freezing at which time the last shrinkage would occur in the runner itself and the entire 90 ingot in the mold is solid non-segregated steel.

95 Referring now to the drawings the mold may comprise a pair of mold members 1 and 2 which are preferably separated on a vertical plane of separation and with relatively heavy heat absorbing walls 4 on all sides of the mold matrix 5. The top and bottom edges of the mold members may be provided with clamping lugs 6 over which C-clamps 7 are adapted to be driven in order to hold the mold members together during the pouring operation. The mold members are provided at one end with recesses 8 and 9 which extend at right angles across one end of the mold matrix and which are of a combined

100 105 110 115 120 125 130

width substantially that of the cross-section of the matrix. These recesses are adapted to receive a suitable runner tile 10. This runner tile is preferably a combined runner tile and fountain and is provided with a body portion 11 and a fountain portion 12. The body portion is provided with a vertical conduit 14 which terminates in a lower inlet opening 15 and leads upwardly to the funnel 16 of the fountain. This funnel preferably extends downwardly into the body portion of the runner sufficiently so that the upper inlet opening 17 is substantially within the lower end of the fountain whereby hot steel is continually fed to the upper opening without danger of the conduit being choked at this point. Preferably the openings 15 and 17 are so proportioned as to cross-sectional area that the steel issuing from the lower opening will be substantially the same volume per unit of time as is the steel issuing from the upper opening. When the fountain is kept filled with steel, obviously the pressure at the lower opening is greater than at the upper opening, therefore during the same interval more steel will issue through the lower opening than through the upper opening, unless the areas are respectively proportioned to counterbalance the pressure conditions. The ends of the mold members may be provided with crane knobs 18 to facilitate the lifting of the mold members and the bottoms of the mold members may be provided with suitable legs 19 and 20 to maintain the axis of the matrix slightly inclined to the horizontal, with the inclination toward the gas outlet in the mold body.

Figure 2 illustrates by means of arrows the churning or stirring action which occurs due to the arrangement of the pouring openings, and arrows A illustrate the substantially horizontal direction of the steel spouting from the lower opening 15, whereas the arrows B illustrate the downwardly direction of the steel issuing from the upper opening 17 and the arrows C indicate the swirling or mixing action in a vertical direction which occurs in the steel in the mold during the pouring operation. This action effectively prevents segregation. Preferably a gas outlet opening 21 is provided between the mold body and the runner tile adjacent the fountain portion of the tile. This facilitates escape of gases from the mold during pouring.

Referring more specially to Figure 3 which shows the condition immediately after freezing and which illustrates the manner in which the ingot shrinks in the mold, it will be noted that in view of the fact that the end farthest from the runner cools first, the majority of shrinkage appears to be at this end and the space as at D is formed between the end of the ingot and the mold wall. A wedge shaped space E is also formed between the upper side walls of the mold and

the ingot. A slight shrinkage pipe F may form in the fountain 12, but the body of the ingot is solid steel.

In carrying out the method of the present invention the tile 10, which is composed of fire clay preferably of porous texture and having a large heat absorbing capacity, is heated as hot as possible. The hot runner tile is then set in the recesses in the end of the mold body and the steel is poured as quickly as possible after the setting of the hot runner so that the mold is filled with molten steel before the runner has cooled to any appreciable extent. As the steel enters the matrix the churning action specified occurs and there is no liability of the constituents of the alloy segregating. The mold is filled as quickly as possible and the chilling action beginning at the far end of the mold proceeds toward the hot runner tile which continues to feed molten steel as is required to fill any cavities tending to form due to shrinkage. The final result is what is known in the art as a "perfect ingot" which is adapted to be fabricated as an entirety into commercial forms.

Having thus described my invention, what I claim is:

1. The method of manufacturing ingots from dead melted steel in a horizontal covered mold matrix, comprising positioning a preheated wall adjacent one end of the mold matrix and introducing molten steel into the mold matrix through an opening in the hot wall and in sufficient volume to quickly fill the matrix before the hot wall is cooled to an appreciable extent.

2. The method of manufacturing ingots from dead melted steel in a horizontal covered mold matrix, comprising positioning a hot vertical wall to comprise a vertical end of the mold matrix and introducing molten steel into the mold matrix adjacent the hot wall in sufficient volume to quickly fill the matrix before the hot wall is cooled to an appreciable extent.

3. The method of manufacturing in chill molds ingots from dead melted steel, comprising positioning a hot vertical wall to comprise a vertical end of the mold matrix and introducing molten steel into the mold matrix through an opening in the hot wall and in sufficient volume to quickly fill the matrix before the hot wall is cooled to an appreciable extent while chilling the remaining sides of the ingot.

4. The method of casting horizontal ingots from dead melted steel, comprising positioning a hot wall adjacent the inlet of the steel to the mold cavity, chilling all other portions of the mold cavity, and causing freezing of the steel to progress from the portion of steel farthest from the inlet toward the inlet while the said wall is maintained hot.

5. The method of casting horizontal ingots from dead melted steel, comprising utilizing a hot vertical wall as the inlet for the steel to the mold cavity, causing the molten steel to enter the mold in a horizontal direction and to have eddy currents in a vertical direction, chilling all other portions of the mold cavity, and causing freezing of the steel to progress from the portion of steel farthest from the inlet toward the inlet while the said vertical wall is maintained hot. 70
6. The method of casting horizontal ingots from dead melted steel which comprises utilizing a completely covered chill mold, inclining the mold to the horizontal, maintaining a hot wall adjacent the high end of the mold matrix, and introducing the steel into the mold matrix adjacent the hot wall. 75
7. The method of casting steel ingots in a covered chill mold, which comprises positioning a hot runner tile to form substantially one vertical wall of the mold matrix and introducing the steel into the matrix through said hot runner tile. 80
8. The method of casting steel ingots which comprises preheating a runner tile adjacent one wall of a horizontal closed chill mold and introducing a plurality of horizontal streams of steel into the matrix through said hot runner tile. 85
9. The method of casting steel ingots in a cold covered horizontal chill mold, which comprises positioning a highly heated runner tile vertically at one end of said mold in such manner that the runner tile comprises substantially the end wall of said mold and filling said mold from said hot runner tile through openings to cause a mixing action of the steel as it fills the mold matrix. 90
10. The method of casting steel ingots in a cold covered chill mold, which comprises positioning a highly heated runner tile at one end of said mold in such manner that the runner tile comprises substantially the end wall of said mold, and filling said mold from said hot runner tile through openings having horizontal axes one over the other to cause a mixing action of the steel as it fills the mold. 95
11. The method of casting steel ingots in a cold covered chill mold, which comprises positioning a highly heated runner tile at one end of said mold in such manner that the runner tile comprises substantially the end wall of said mold and filling said mold from said hot runner tile, and maintaining a vertical mixing action in the steel in the mold until the matrix is filled. 100
12. The method of casting a steel ingot which comprises casting the ingot in a horizontal full chilled mold, utilizing a heated inlet conduit to prevent the supply stream of molten steel from freezing, causing agitation in the steel to prevent segregation during pouring, then causing the steel to freeze as soon as possible after the mold is filled. 105
13. The method of casting a steel ingot which comprises casting the ingot in a horizontal full chilled mold, utilizing a heated inlet conduit to prevent the supply stream of molten steel from freezing, causing agitation in the steel to prevent segregation during pouring, then causing the steel to freeze as soon as possible after the mold is filled with the heat gradient running toward the hot conduit so that the steel in the conduit is last to solidify. 110
14. The method of casting a steel ingot which comprises casting the ingot in an inclined horizontal full chilled mold, utilizing a heated inlet conduit to prevent the supply stream of molten steel from freezing, pouring the steel into one end of the mold matrix, causing agitation in the steel in the matrix to prevent segregation during pouring, then causing the steel to freeze as soon as possible after the mold is filled. 115
15. The method of casting a steel ingot which comprises casting the ingot in a horizontal full chilled mold, utilizing a heated inlet conduit to prevent the supply stream of molten steel from freezing, causing agitation in the steel to prevent segregation during pouring, causing mold gases to issue from the highest portion of the matrix, then causing the steel to freeze as soon as possible after the mold is filled. 120
16. The method of casting a steel ingot which comprises casting the ingot in an inclined horizontal full chilled mold, utilizing a heated inlet conduit to prevent the supply stream of molten steel from freezing, pouring the steel into one end of the mold matrix, causing agitation in the steel in the matrix to prevent segregation during pouring, causing mold gases to issue from the highest portion of the matrix, then causing the steel to freeze as soon as possible after the mold is filled with the heat gradient running toward the hot conduit so that the steel in the conduit is last to solidify. 125
17. The method of casting steel ingots which comprises heating a wall of the mold matrix, filling the mold matrix by introducing molten steel adjacent said wall thereby filling the mold matrix by converging streams of steel, quickly chilling the steel in the matrix when the matrix is full while supplying molten steel through the hot wall as the steel in the mold freezes. 130
18. The method of casting steel ingots which comprises heating a wall of the mold matrix, filling the mold matrix by introducing molten steel adjacent said wall thereby filling the mold matrix by a plurality of converging streams of steel, quickly chilling the steel in the matrix when

the matrix is full and causing the temperature gradient to run toward the hot wall while supplying molten steel through the hot wall as the steel in the mold freezes.

5 19. The method of casting steel ingots which comprises heating a wall of mold matrix, filling the mold matrix by introducing molten steel adjacent said wall thereby filling the mold matrix by horizontally directed converging streams issuing through the hot wall, at the highest part of the matrix, quickly chilling the steel in the matrix when the matrix is full while supplying molten steel through the hot wall 10 as the steel in the mold freezes.

15 20. The method of casting the metallic ingot which comprises preheating an end wall of a horizontal closed chill mold, and filling the mold matrix with molten 20 metal in substantially horizontal streams from the preheated end before the latter has cooled.

25 21. The method of casting a metallic ingot which consists in preheating a heat retaining wall forming the major portion of an end of a horizontal covered mold matrix and then introducing the molten metal adjacent said wall to fill the matrix before the wall has cooled.

30 22. The method of casting a metallic ingot which consists in preheating a heat retaining wall forming an end of a horizontal covered mold matrix and then introducing the molten metal through said wall in 35 converging streams to fill the matrix before the wall has cooled.

35 23. The method of casting a metallic ingot which consists in preheating a heat retaining wall forming a major portion of an end of a horizontal covered mold matrix, and then introducing the molten metal through said wall with a mixing action to fill the matrix before the wall has cooled.

40 24. The method of casting a metallic ingot which consists in preheating a heat retaining wall forming an end of a horizontal covered mold matrix and then introducing the molten metal adjacent said wall with a mixing action to fill the matrix before the wall has cooled to an appreciable extent.

45 25. The method of casting metallic ingots which consists in preheating a heat retaining wall at the inlet end of a horizon-

tal closed chill mold, introducing the molten metal adjacent said wall in a horizontal direction with eddy currents substantially in a vertical direction and chilling the outer portions of the mold whereby the freezing of the metal progresses toward said wall 55 while the latter is maintained hot.

5 26. The method of casting ingots which comprises preheating the insulating end wall of a horizontal matrix, simultaneously directing a plurality of streams of molten metal into the matrix through a plurality of orifices in the preheated end wall to cause a mixing action within the mold and chilling the top, bottom, sides and the end of the confined metal while the head end is in relatively molten condition.

70 27. The method of casting horizontal steel ingots, which comprises preheating an end wall of a horizontal closed chill mold and filling the mold with molten metal 75 through the preheated end thereof before the latter has cooled materially.

75 28. The method of casting horizontal ingots which comprises preheating a heat retaining wall in a horizontal covered mold, introducing molten metal adjacent said wall, mixing the metal within the mold and delaying the chilling of the ingot at the entrance end of the mold until after all of the remaining surfaces have been chilled.

80 29. The method of casting horizontal ingots which comprises preheating the runner tile at one end of a horizontal chill mold and filling the mold matrix through said runner tile before said tile has cooled 85 appreciably.

85 30. The method of casting ingots in a horizontal covered mold matrix, which comprises placing a hot wall adjacent one end of the horizontal mold and introducing molten steel into the mold matrix adjacent the hot wall to fill the matrix before the hot wall cools to an appreciable extent.

90 31. The method of casting ingots in a horizontal covered mold matrix which comprises mounting a hot member adjacent one end of the mold matrix and introducing molten metal into the mold matrix adjacent the hot member in sufficient volume to quickly fill the matrix before the hot member is cooled to an appreciable extent.

100 EDWARD H. WILLIAMS.